

## UNITED STATES PATENT OFFICE

2,058,421

## TEXTILE MATERIAL

William Alexander Dickie and Robert Wighton  
Moncrieff, Spondon, near Derby, England, as-  
signors to Celanese Corporation of America, a  
corporation of Delaware

No Drawing. Application April 2, 1931, Serial No.  
527,358. In Great Britain May 7, 1930

10 Claims. (Cl. 28—1)

This invention relates to the manufacture of textile fabrics exhibiting crêpe effects.

Textile fabrics exhibiting crêpe effects have long been obtained by employing in their con-

5 5 construction highly twisted yarns, hereinafter referred to as crêpe yarns or crêpe threads, made of natural silk in the gummed state, the crêpe effects appearing when the gum is subsequently removed by scouring or like treatment. The production of crêpe effects by the employment of highly twisted crêpe threads made of cellulose acetate or other organic derivatives of cellulose has however been accomplished with consider-

10 10 We have now found that crêpe effects may be produced upon fabrics containing highly twisted crêpe threads by processes comprising the application of concentrated solutions of organic or inorganic salts. We have found for example that 15 20 a fabric containing highly twisted crêpe threads of cellulose acetate filaments may be caused to exhibit crêpe effects by treatment with a concentrated solution of calcium chloride followed by a scouring or like aqueous treatment.

25 25 The invention is of special value in the production of crêpe effects upon fabrics containing highly twisted crêpe threads made with filaments of cellulose acetate or other organic derivatives of cellulose and will therefore be described more particularly with reference to such fabrics.

30 30 Either organic or inorganic salts capable of yielding concentrated solutions in water or other liquids may be employed for the purposes of the present invention. As examples of such salts may be mentioned the halide salts of alkaline earth metals or of lithium or zinc, for example the chlorides of lithium or zinc, in addition to calcium chloride mentioned above. Other wholly inorganic salts which may be used are the acid 35 40 alkali-metal salts of di- or polybasic acids, for example sodium hydrogen sulphate or sodium dihydrogen phosphate. As example of salts of inorganic bases with organic acids may be instanced the alkali metal salts of acetic acid or other aliphatic acids, for example sodium or potassium acetate. Further salts of organic bases may also be employed, for example methylamine hydrochloride.

45 50 Especially good results may be obtained with the aid of concentrated solutions of salts which are deliquescent or hygroscopic or have a marked affinity for water, for example calcium chloride, zinc chloride, or sodium or potassium acetate.

55 55 The solutions, preferably aqueous, may be of

such high concentration as to be capable of taking up water readily, for example from the atmosphere or from the materials under treatment.

It appears that the concentrated salt solutions 5 do exert a dehydrating action on the material of the crêpe threads which when allowed to absorb water again, tend to diminish in length and give rise to the desired crêpe effects.

Indeed it has further been found that the concentrated salt solutions may be replaced for the purposes of the present invention by other agents or treatments having a dehydrating action on the material of the crêpe thread filaments. For example the fabrics may be treated with ethyl or 15 methyl alcohol, either absolute or containing a small proportion of water, the alcohol removed by drying in the absence of moisture, and the fabrics finally treated with water.

Again the fabrics may be dehydrated by boiling 20 with benzene or other suitable liquid, in order to remove water as an azeotropic mixture therewith.

The fabrics containing highly twisted crêpe threads made of or containing organic derivatives of cellulose may, after subjection to treatment with a concentrated solution of a salt or to another dehydrating treatment as already indicated, be subjected to the action of water in any desired manner. For example the fabrics may be 25 30 washed in water or scoured in an aqueous scouring bath, preferably such as is stable in the presence of any salts utilized. Water is thus absorbed and the desired crêpe effects produced or accentuated.

If desired water may be applied in restricted 35 40 quantity to the dehydrated materials, in many cases with advantage. Thus the materials may be treated with water vapour, e. g. in the form of air or other gas laden with water vapour, for such time as may be necessary to secure maximum development of the desired crêpe effect. Again the materials may be sprayed with water in quantity no greater than is necessary to effect 45 50 production of the crêpe effects for example in quantity of from 10 to 40 per cent. of the weight of the materials. After spraying with the requisite proportion of water or other aqueous liquid, the materials may be allowed to stand to permit the water to exert its effect, e. g. the material may be rolled up and left for a time.

The concentrated salt solutions may be applied to the fabrics containing highly twisted crêpe threads in any convenient manner and either uniformly or otherwise as desired. For example in 55

the case of uniform application the materials may be passed through the concentrated salt solutions, or more conveniently, they may be padded with the solutions, e. g. by means of a padding mangle. If desired, the concentrated salt solutions may be applied locally to the materials, for instance by printing or stencilling, whereby brocade or like effects may be produced. Salt solutions to be applied locally or by padding may 10 be suitably thickened if desired or requisite.

The concentrated salt solutions may be permitted to remain in contact with the materials for a substantial time depending on the nature of the salts used, the concentration and temperature of the solutions, and the nature of the materials under treatment. To this end the materials may be allowed to remain for a time in the baths when these are employed, or when the salt solutions have been applied by padding 20 the materials may be batched, that is to say they may be rolled or otherwise parcelled up and allowed to stand until the salt solutions have acted on the materials for a sufficient time.

It will be appreciated that the nature, temperature, and time of action of the salt solutions or other dehydrating agents should not be such as to cause damage to the materials.

According to a modification of the invention the crêpe threads may be subjected to the action of concentrated salt solutions or a dehydrating treatment prior to weaving or even prior to the application of the requisite high degree of twist. The yarns to serve as crêpe threads may for instance be passed through the concentrated salt solutions in transit to a twisting device for the application of the requisite twist. The highly twisted yarn may then be incorporated in fabrics and the latter subjected to an aqueous treatment.

40 The degree of twist imparted to the yarns or threads of cellulose acetate or other organic derivatives of cellulose serving to give the crêpe effects may be similar to that commonly employed in the production of crêpe threads from natural silk, for example the threads may have imparted thereto a twist of from 50-75 turns per inch. Any other suitable degree of twist may however be employed according to the effects it is desired to produce. If desired, two or more highly twisted threads of the same or different direction or degree of twist may be doubled together to form the crêpe threads. By suitable variation of the component threads, degree of twist, etc. a wide variety of effects may be produced.

55 The highly twisted crêpe threads may be incorporated in the fabrics in any suitable manner, for example the weft alone may be wholly or partially composed of such threads or the warp may also contain them. In the former case on treatment in accordance with the invention, the fabrics exhibit chiefly shrinkage in the direction of the weft. It is found most convenient in general to employ threads of relatively low twist in the warp and to employ in the weft both crêpe threads having a left-hand twist and crêpe threads having a right-hand twist. Threads having left- and right-hand twist respectively may be disposed in the fabric in any convenient manner. For example pairs of 60 threads of left-hand twist may alternate with pairs of threads of right-hand twist.

The crêpe threads used in producing fabrics in accordance with the present invention may be made of or contain filaments of any desired 65 organic derivatives of cellulose, for example cel-

lulose esters, e. g. cellulose acetate, formate, propionate or butyrate, or cellulose ethers, e. g. ethyl, methyl or benzyl cellulose, or the analogous condensation products derived from cellulose and glycols or other polyhydric alcohols. The fabrics may be composed wholly of yarns made of or containing organic derivatives of cellulose, or they may comprise also yarns of other filaments or fibres whether natural or artificial. As examples of other fibres may be mentioned artificial silk of the regenerated cellulose type and also cotton, wool or silk or other natural fibre. 10

Though the invention has been described more particularly with reference to the manufacture of crêpe fabrics containing crêpe threads made with filaments of cellulose acetate or other organic derivatives of cellulose the invention is not limited to the use of such crêpe threads. As previously indicated crêpe threads made with filaments of other materials, for example degummed silk, regenerated cellulose, or other natural or artificial materials may likewise be utilized.

Crêpe threads may also be employed composed of filaments of two or more different kinds, 25 whether in respect of material or size or both. Thus there may be used threads containing both filaments of cellulose esters or ethers and filaments of regenerated cellulose or natural silk, or threads containing cellulose ester or ether 30 filaments of two or more different deniers.

Further, the crêpe threads, whether made from filaments of organic derivatives of cellulose or natural or artificial filaments or fibres of other materials, may be sized prior to twisting and/or 35 weaving. In such case the treatment with concentrated solutions of salts and/or the washing, scouring, or other subsequent treatment may be adapted to swell the sizing materials thereon. Where the production of the crêpe effects is 40 dependent, wholly or in part, upon a swelling of a sizing material, the latter may be selected and applied so that the size may be caused to swell by the treatment with the salt solutions and/or other treatment without becoming unduly 45 soft or yielding. Further it is advisable that the filaments of the crêpe threads be coated individually with size. In order that this may be the case the crêpe threads may be sized prior to twisting or at least prior to the application of 50 a high degree of twist, or if desired the filaments may be sized singly or in comparatively small groups, prior to their being brought together to form a thread of the required thickness.

The invention is illustrated but not limited by 55 the following examples:—

#### Example 1

A fabric comprising a warp of cellulose acetate 60 yarns of low twist and a weft of cellulose acetate 65 yarns twisted to 65 turns per inch is padded with a 30% to 40% solution of calcium chloride. After standing for a time say 1/2-2 hours, the material is washed well in warm water to which a sulphonated oil stable in presence of calcium chloride 70 may be added. The fabric is finally dried without tension. In like manner concentrated solutions of other salts for example sodium or potassium acetate may be employed.

#### Example 2

A fabric composed of cellulose acetate yarns of the kind described in Example 1 is treated for half an hour with warm absolute ethyl alcohol and is then freed from alcohol and carefully 75

dried in the absence of moisture. The fabric is then passed through a chamber in which it is treated with a mist or finely divided spray of warm water, the latter being supplied in quantity about 30 to 40 per cent. of the weight of the fabric.

*Example 3*

A cellulose acetate fabric of the kind referred to in Example 1 is treated locally with a saturated solution of calcium chloride, the latter being applied by spraying through stencils. After standing for a short time the material is rapidly washed in a large volume of warm water and dried.

*Example 4*

A fabric made entirely from cellulose acetate yarn of 75 denier and 70 turns per inch in which two threads of left-hand twist yarn alternate with two threads of right-hand twist yarn in both warp and weft, is immersed in a saturated solution of sodium hydrogen sulphate. The fabric is then rinsed, scoured and dyed and finally dried without tension.

*Example 5*

Cellulose acetate yarn of 140 denier and of low twist is passed through a strong solution of calcium chloride at ordinary temperature. The yarn is then twisted to 55 turns per inch and woven into a cotton warp, two picks of yarn of left-hand twist alternating with two picks of yarn of right-hand twist. The resulting fabric is thereafter scoured and finally dried without tension.

What we claim and desire to secure by Letters Patent is:—

1. In a production of textile fabrics exhibiting crepe effects in which yarns are twisted to a high degree and incorporated in fabrics and the latter subjected to an aqueous treatment, the step of subjecting the yarns to the action of a dehydrating reagent prior to the incorporation of the yarns in the fabrics.

2. In a production of textile fabrics exhibiting crepe effects in which yarns containing filaments of organic derivatives of cellulose are twisted to a high degree and incorporated in fabrics and the latter subjected to an aqueous treatment, the step of subjecting the yarns to the action of a dehydrating reagent prior to the incorporation of the yarns in the fabrics.

3. In a production of textile fabrics exhibiting crepe effects in which yarns containing filaments of cellulose acetate are twisted to a high degree and incorporated in fabrics and the latter subjected to an aqueous treatment, the step of subjecting the yarns to the action of a dehydrat-

ing reagent prior to the incorporation of the yarns in the fabrics.

4. Process for the production of crepe effects upon fabrics containing crepe twisted yarns of filaments of organic derivatives of cellulose, which comprises subjecting the yarns to the action of a concentrated solution of a salt having good affinity for and high solubility in water, and thereafter incorporating said yarns into fabrics and subjecting the fabrics to an aqueous treatment.

5. Process for the production of fabrics exhibiting crepe effects which comprises treating yarn containing filaments of organic derivatives of cellulose with concentrated solutions of salts having good affinity for and high solubility in water, imparting a crepe twist to the yarn, incorporating the yarn in fabrics and subjecting the fabrics to an aqueous treatment.

6. Process for the production of fabrics exhibiting crepe effects which comprises treating yarn containing cellulose acetate filaments with concentrated solutions of salts having good affinity for and high solubility in water, imparting a crepe twist to the yarn, incorporating the yarn in fabrics and subjecting the fabrics to an aqueous treatment.

7. Process for the production of crepe effects upon fabrics containing crepe twisted yarns of filaments of organic derivatives of cellulose, which comprises subjecting the yarns to the action of a concentrated solution of an alkali metal acetate, and thereafter incorporating said yarns into fabrics and subjecting the fabrics to an aqueous treatment.

8. Process for the production of fabrics exhibiting crepe effects which comprises subjecting yarns of low twist to the action of a dehydrating reagent, applying a crepe twist thereto, incorporating the crepe-twisted yarns in fabrics, and subjecting the fabrics to an aqueous treatment.

9. Process for the production of fabrics exhibiting crepe effects which comprises subjecting yarns of low twist containing filaments of organic derivatives of cellulose to the action of a dehydrating reagent, applying crepe twist thereto, incorporating the yarns in fabrics and subjecting the fabrics to an aqueous treatment.

10. Process for the production of fabrics exhibiting crepe effects which comprises subjecting yarns of low twist containing filaments of cellulose acetate to the action of a dehydrating reagent, applying crepe twist thereto, incorporating the yarns in fabrics and subjecting the fabrics to an aqueous treatment.

WILLIAM ALEXANDER DICKIE. 55  
ROBERT WIGHTON MONCRIEFF.